

(No Model.)

2 Sheets—Sheet 1.

H. FRASCH.

ELECTRIC CARBON.

No. 281,048.

Patented July 10, 1883.



WITNESSES

Jas. E. Hutchinson.  
George Cook

INVENTOR

Herman Frasch.  
By Saggett & Saggett  
Attorney

(No Model.)

2 Sheets—Sheet 2.

H. FRASCH.  
ELECTRIC CARBON.

No. 281,048.

Patented July 10, 1883.

Fig. 3.



Fig. 4.



WITNESSES

Jas. E. Hutchinson.  
George Cook.

INVENTOR

Hermann Frasch.  
By Segget & Segget  
Attorney

# UNITED STATES PATENT OFFICE.

HERMAN FRASCH, OF CLEVELAND, OHIO, ASSIGNOR TO J. B. MERIAM, OF SAME PLACE.

## ELECTRIC CARBON.

SPECIFICATION forming part of Letters Patent No. 281,048, dated July 10, 1883.

Application filed January 12, 1883. (No model.)

*To all whom it may concern:*

Be it known that I, HERMAN FRASCH, of Cleveland, in the county of Cuyahoga and State of Ohio, have invented certain new and useful 5 Improvements in Electric Carbons; and I do hereby declare the following to be a full, clear, and exact description of the invention, such as will enable others skilled in the art to which it pertains to make and use it, reference being had to the accompanying drawings, which form part of this specification.

My invention relates to the manufacture of carbon especially adapted for use in making electric-light carbon rods or sticks; and it consists in a process for the manufacture of carbon from the products of petroleum, and also in process for preparing a carbon mixture for molding into any desired shape, as will herein-after be described, and pointed out in the 20 claims.

Heretofore carbon has been obtained in the distillation of petroleum from carbon residuum when the latter has been reduced to dryness; but such carbon is a decomposition product, 25 and is limited to the quantity obtained in the distillation of petroleum. My object is to obtain from hydrocarbon oils practically all of the carbon contained therein, and thus need not be restricted to the small percentage eliminated in the destructive distillation of petroleum.

In the accompanying drawings, Figure 1 is a front elevation. Fig. 2 is a plan view. Fig. 3 is a transverse section, and Fig. 4 is a longitudinal vertical section.

A represents the ash-pit, and B the fire-box door. The ash-pit communicates with two flues, C C', which extend to the rear end of the furnace, and then back and forth, forming 40 turn-flues, and having their exit in the escape-flues D D' at the front of the furnace, where they merge into the stack or chimney E. The hearth of the furnace is constructed of the tilings a, which are placed directly over the flues C C'. Upon the tilings a is placed a layer of asbestos, b, and upon the latter are placed the tilings c, which are laid to break joints with the lower tilings, a. The arch F is covered with sand d and the walls strengthened by the rods 45 e. At the front of the furnace is located the

charging-opening G, provided with a door, G'. This door is located at a sufficient distance above the hearth or floor of the furnace to allow of the proper charging of the furnace. At the sides and end of the furnace are the 55 doors H, which are placed on a level with the hearth or floor for the removal of the carbon. An escape-pipe, I, communicates with the upper portion of the furnace-chamber, and is provided with a stop-cock or valve, i. A pipe, J, 60 connects with the pipe I, and leads beneath the grate of the fire-box. Pipe J is provided with a stop-cock or valve, j. The lower end of the chimney or stack is provided with a damper, K.

Having described the construction and relative arrangements of my improved furnace, I will now describe its operation.

I take distilled hydrocarbon of high density obtained by the distillation of petroleum or other hydrocarbon oils, and mix the same with 70 sulphuric or nitric acid. After the furnace has been heated, all of the doors being closed, the charging-door is opened and the compound is charged into the furnace to the proper depth. When the temperature reaches about 300° 75 Fahrenheit, the mass being quite liquid, reaction begins to take place, the hydrogen of the hydrocarbon combining with the oxygen of the acid, if sulphuric be used, or steam and nitrogenous compounds when nitric acid is used. This 80 reaction tends to stiffen the whole mass, so that it becomes quite hard even before the temperature of 500° Fahrenheit is reached. By continuing the operation and gradually increasing the temperature to, say, 1000° Fahrenheit or 85 more, all of the decomposition products, being volatile, are driven off, leaving a carbon coke upon the hearth of the furnace almost chemically pure, quite dense and dry, and easily removed, which is effected by opening the side 90 doors and inserting a slice-bar beneath the mass, breaking it up into pieces and removing them through the side doors. In charging the furnace the damper K is opened to conduct the escaping flame into the chimney, and thus 95 not interfere with the workmen. The gases generated in the furnace may be allowed to escape or be conducted to the ash-pit and burned. The quantity of coke obtained by the process described is a large percentage of the 100

carbon originally employed. The sludge oils and acid compounds which are drawn off in the ordinary treatment of petroleum distillates may be subjected to the same treatment, in which case the same reaction takes place and the same carbon product is obtained, thereby very profitably utilizing what have heretofore been regarded as the waste products of an oil-refinery. The furnace is so constructed that the heat will be evenly distributed beneath the hearth, and the latter is made comparatively thin, so that the heat may be readily transmitted to the charge. By means of the two layers of tilings arranged to break joints and the intervening layer or packing of asbestos a perfectly-tight hearth or floor is insured.

In the preparation of this carbon for electric-light carbon rods or sticks, I first grind it to a suitable degree of fineness and then mix the powder with a paste consisting of the very dense products of distillation of petroleum-tar or residuum known as "wax-tailings" or "still-wax," which come over just after the so-called "paraffine-oils" and during the coking down of the still. This compound can then be molded and baked in the usual manner. The advantage in the use of the paste over that of ordinary pitch consists in its freedom from impurities, for, having passed through a vapor state, it is a pure hydrocarbon, free from matters leaving ash, the impurities of the crude petroleum being retained in the still; where-

as the pitch ordinarily used is the residuum from coal-tar and a small percentage of the same, and contains all the impurities of the coal-tar concentrated. These wax-tailings may be still further improved by driving off the lighter portions by partial distillation.

I make no claim to the construction of furnace herein shown and described, as it constitutes the subject-matter of a separate application; but

What I claim is—

1. The process of manufacturing carbon from hydrocarbon compounds, consisting in oxidizing the hydrogen of the hydrocarbon by heating a mixture of the hydrocarbon and an acid to such a degree that decomposition takes place, and continuing the same until all the decomposition products are driven off, leaving a solid carbon as a residuum, substantially as set forth.

2. An incandescent composition consisting of a mixture of pulverized carbon and the heavy distillate obtained in the distillation of petroleum known as "wax-tailings" or "still-wax," or with a product of the same, substantially as set forth.

In testimony whereof I have signed my name to this specification in the presence of two subscribing witnesses.

HERMAN FRASCH.

Witnesses:

JNO. CROWELL, Jr.,  
ALBERT E. LYNCH.